

June 7, 1938.

U. B. BRAY

2,120,209

## METHOD FOR SOLVENT EXTRACTION OF OIL

Filed March 21, 1934



INVENTOR.  
*Ultric B. Bray*  
BY *Philip Subkow*  
ATTORNEY.

## UNITED STATES PATENT OFFICE

2,120,209

METHOD FOR SOLVENT EXTRACTION OF  
OIL

Ulric B. Bray, Palos Verdes Estates, Calif., assignor to Union Oil Company of California, Los Angeles, Calif., a corporation of California

Application March 21, 1934, Serial No. 716,581

6 Claims. (Cl. 196—13)

This invention relates to a process for the treatment of petroleum with selective solvents. Although it may be employed for use with other petroleum fractions, it is especially applicable to the treatment of lubricating oil.

In the production of lubricating oil for internal combustion motors it is highly desirable to obtain a product which exhibits a low temperature viscosity susceptibility, a low Conradson carbon residue value, a high stability towards sunlight and a low oxidation value. Crude lubricating oil fractions produced either as distillates or as residues are usually composed of mixtures of paraffinic, naphthenic, aromatic and olefinic hydrocarbons. The olefinic hydrocarbons are highly unsaturated and their presence in the finished lubricating oil is undesirable because of their unstable characteristics. These compounds are unstable and usually darken when exposed to sunlight. Furthermore, they have a high tendency towards polymerization with the result, after a considerable period, that these compounds are converted into resinous substances which increase the sludge value of the oil.

The aromatic and naphthenic hydrocarbons present in crude lubricating oil fractions are undesirable because these compounds exhibit too great a change in viscosity for a given change in temperature. The paraffinic hydrocarbons present in crude lubricating oil fractions are the most desirable materials to be employed as lubricants. These compounds are highly saturated hence, from a chemical standpoint, they are rather inactive and do not exhibit a tendency towards the formation of undesirable resinous or sludge-forming constituents. Furthermore, these compounds exhibit a low temperature viscosity susceptibility. In other words, they exhibit a minimum change in viscosity for a given change in temperature. Furthermore, these highly saturated hydrocarbons are relatively stable to sunlight, exhibiting little tendency toward discoloration or sludge formation. When I use the term "paraffinic hydrocarbons" I mean those compounds which are present in petroleum having the aforementioned characteristics and which are liquid at ordinary temperatures. This group of hydrocarbons does not include those compounds present which are usually solid or semi-solid at ordinary temperature and which are known as "wax" or "petrolatum".

A further indication of the purity of a lubricating oil is its viscosity gravity constant. This constant represents the paraffinicity or naphthenicity of an oil. A high value represents a

high degree of naphthenicity while low values indicate relatively greater paraffinicity. Lubricating oils from natural crudes range from 0.903 viscosity gravity constant for an extreme Gulf Coast type to 0.807 for an extreme Pennsylvania type, or even beyond. The viscosity gravity constant referred to in this application has been determined by the method employed by Hill and Coates as set forth in the Journal of Industrial and Engineering Chemistry, vol. 20, page 641 of 1928.

As a matter of convenience hereafter I will refer to those constituents of petroleum characterized by relatively low viscosity gravity constant as the "paraffinic" hydrocarbons, and to those constituents of petroleum characterized by relatively high viscosity gravity constant, as the "non-paraffinic" constituents of petroleum.

In the production of lubricating oil from crude petroleum residues or distillates, it is becoming conventional in the art to separate the desirable paraffinic hydrocarbons from the undesirable olefinic, naphthenic and/or aromatic compounds by the use of solvents which selectively dissolve the undesirable hydrocarbons present in the petroleum fraction but which exhibit only a very limited solvent power on the desirable paraffinic hydrocarbons.

A number of selective solvents have been found desirable to separate the paraffinic from the non-paraffinic hydrocarbons, for example, it has been shown that such materials as sulphur dioxide, beta beta dichlorethyl ether, chloraniline, nitrobenzene, aniline and furfural are highly selective as the solvents for the non-paraffinic hydrocarbons. The foregoing selective solvents are relatively heavy as compared to petroleum. When these relatively heavy solvents are commingled with petroleum or petroleum fractions under the proper conditions of temperature, the undesirable non-paraffinic hydrocarbons present pass into solution to a greater or less extent but the desirable paraffinic hydrocarbons remain largely undissolved. If the commingled mass is allowed to remain in a quiescent state the solution of undesirable hydrocarbons and solvent settles to the bottom of the container and forms what is known as an "extract" phase. The relatively light paraffinic hydrocarbons rise to the top of the vessel and form a raffinate phase. These phases are then readily separable by ordinary decantation means. The raffinate phase is usually found to contain a small quantity of the selective solvent and the extract phase ordinarily contains a relatively large quantity of

the solvent. These fractions may be purified by subjecting them to distillation whereby the solvent is distilled away from the hydrocarbon oils.

Due to the general similarity of the various hydrocarbon components of mineral oil fractions such as lubricating oils, solubilities of the undesirable, non-paraffinic fractions and the desirable paraffinic fractions in a selective solvent usually differ only in degree, and there is, therefore, a tendency for desirable, high grade paraffinic oil to be carried away with the extract resulting in a loss in the yield of paraffinic fractions obtained. In other words, in a phase separation of extract and raffinate fractions from mineral oil employing a selective solvent, an equilibrium of paraffinic components as well as non-paraffinic components is established between the phases. Consequently, some of the desirable paraffinic fraction is found in the extract instead of in the raffinate.

While some loss may occur in a primary extraction of lubricating oil with a selective solvent for the production of a low grade primary extract and a primary raffinate, the loss of desirable paraffinic fractions in the extract is especially severe when the raffinate produced by the primary extraction is further treated by a selective solvent to produce a high grade raffinate and an intermediate grade extract. In the production of a low grade primary extract and a primary raffinate in the first extraction, the difference in solubility of the respective oils is usually so great that commercially satisfactory separation is obtainable. In some cases, however, such a process results in a substantial loss of paraffinic components in the low grade extract. The difference in solubility between the intermediate grade extracts and high grade raffinate produced by a succession of extractions is usually not so great and there is, therefore, more tendency for paraffinic oil to be carried away with the intermediate grade extracts.

It has been proposed to regulate the solvent power of the extracting agent at any stage of the treatment in accordance with the solubility of the material to be extracted and as the refining of the stock by extraction progresses in a step-wise manner, the solvent power of the treating agent may be increased.

By substantially increasing the solvent power or ease of miscibility of the treating agent, it is possible to fractionate the raffinate obtained after extraction with the pure solvent into a further extract of lower solubility than the first extract obtained by the use of said pure solvent and a second raffinate of consequently lower solubility than the first raffinate. This may be accomplished by first extracting a hydrocarbon mixture with a pure selective solvent, for instance one of the solvents set forth above, and then to retreating the raffinate so produced with a modified solvent. As modifying agents such materials as carbon bisulphide, xylene, benzene, toluene, carbon tetrachloride, ethers or tetrachlorethane may be employed with the selective solvent.

By these processes the oil feed is divided in one general operation into three or more fractions of different viscosity gravity constants. As previously stated, the successive extractions produce a high grade raffinate and intermediate grade extracts characterized by solubilities which are not very different from each other. Consequently, in ordinary treatment of mineral oil by successive extractions, a substantial portion of the paraffinic fraction is soluble in the extract-solvent mixture

and is lost therein, resulting in a corresponding loss in yield of desirable high grade raffinate.

It has also been proposed to regulate the solvent power of the extracting agent at any stage of the treatment by controlling the temperature at which the extraction takes place. For instance, the temperature at which the primary extraction takes place may be relatively low in order to reduce correspondingly the solvent power of the solvent. The low grade extract thus produced may then contain substantially only the highly aromatic and most soluble fractions of the mineral oil. Subsequent to recovery of the primary raffinate from the low grade extract, the former may again be solvent extracted at a higher temperature than that which prevailed in the primary extraction. The extraction at higher temperature may be accomplished by the same solvent as that used in the primary extraction or a solvent of greater or less solvent power than that employed for the first extraction may be used for the second extraction. These successive extractions likewise produce a high grade raffinate and intermediate grade extracts having relatively similar solubilities and consequently substantial quantities of desirable paraffinic components are lost in the extract phases. Such loss also occurs when mineral oil is successively extracted with the same solvent at the same temperature.

It is an object of my invention to retain the desirable, high grade paraffinic fractions in the raffinate produced by solvent extraction of mineral oils.

The paraffinic fractions may be retained in the raffinate by rectifying the phases. This may be accomplished in a series of successive extractions by intermingling the extract phases with raffinate phases of low content of paraffinic constituents. The equilibrium established in the phase separation of these mixtures is such that the paraffinic content of these extracts tends to be re-distributed into the raffinate phase. When an oil is recovered as a rejected raffinate from the extract phase by cooling, it may be re-introduced into the extraction system for rectification purposes.

I have found that when oil is countercurrently extracted with a selective solvent and the extract phase therefrom is cooled to reject an intermediate raffinate, this intermediate raffinate is characterized by a viscosity gravity constant intermediate that of the raffinate and extract respectively produced by the extraction. It is an object of my invention to aid the rectification of the oil during extraction, and to promote the recovery of paraffinic fractions in the raffinate by introducing this rejected raffinate of intermediate quality into the extraction system preferably into that zone which contains oil of substantially similar characteristics. The equilibrium in the various zones of the countercurrent extraction is thus maintained.

I have also found that when oil is first extracted in a primary extraction zone to produce an extract and a raffinate, and this raffinate is further extracted in a secondary extraction zone to produce a final raffinate and an intermediate extract, that the recovery of valuable paraffinic components in the primary extraction may be augmented by removing the solvent from said intermediate extract phase and returning the intermediate extract into the primary extraction preferably into that zone which contains oil of substantially the same viscosity gravity constant.

Therefore, it is a further object of my inven-

tion to extract an oil with a selective solvent, separate a raffinate insoluble in the solvent from the extract phase, extract the raffinate with a selective solvent to produce a final raffinate and an intermediate extract phase, remove the selective solvent from the intermediate extract phase and introduce the intermediate extract into the first mentioned extraction.

Referring to the drawing, the figure is a diagrammatic view of one type of apparatus suitable for carrying out my invention.

In the apparatus shown in the figure, oil is introduced into primary extractor 10 by pump 11 in line 12 controlled by valve 13. Line 12 connects with orifice mixer 14 which in turn communicates with extractor 10 via line 15. Selective solvent is introduced into extractor 10 by pump 16 in line 17 controlled by valve 18. Extract phase is removed from extractor 10 via line 19 controlled by valve 20. Raffinate phase from 10 passes by action of pump 21 through line 22 controlled by valve 23.

Extractor 10 is divided into a number of sections 26, 27, and 28 by imperforate plates 29. Each section in turn is divided into a mixing zone 30 and a settling zone 31 by plate 32 provided with port 33. Each mixing zone may be provided with an agitator if necessary. I prefer to introduce the selective solvent into the uppermost section 26. Raffinate is removed from this section by line 22 as described. Extract phase from section 26 is removed therefrom by pump 35 through line 36 controlled by valve 37 and is intermixed with the raffinate produced in a lower section of the extractor. This mixture passes through line 38, orifice mixer 39 and line 40 into the mixing zone 30 of section 27. From this mixing zone the mineral oil mixture and solvent passes through port 33 into settling zone 31. The raffinate from the settling zone of section 27 is removed therefrom by action of pump 45 and passes via line 46 controlled by valve 47 into contact with the solvent entering extractor 10 via line 17. This mixture passes through orifice mixer 48 and line 49 into section 26.

The extract phase produced in section 27 is removed by pump 50 through line 51 controlled by valve 52. Line 51 connects with oil feed line 12, and the mixture of extract, solvent and feed passes through orifice mixer 14 and line 15 into section 28 in the manner previously described. The mixture passes through port 33 into settling chamber 31 of section 28 and the raffinate separated therein is passed by pump 53 through line 54 controlled by valve 55. Line 54 joins with line 36 and the commingled material passes through line 38, orifice mixer 39 and line 40 into section 27 in the manner previously described.

Raffinate from extractor 10 passes through line 22, orifice mixer 56 and line 57 into second extractor 60. Extractor 60 is also divided into a number of sections 61 to 65 by plates 29 and each section is divided into a mixing zone 30 and settling zone 31 by plate 32 provided with port 33. Selective solvent is introduced preferably into the upper section 61 of extractor 60 by action of pump 70 in line 71 controlled by valve 72. Line 71 connects with orifice mixer 73 which in turn communicates with extractor 60 via line 74. Extract phase from sections 61, 62, and 63 are removed therefrom by action of pumps 75 through lines 76 controlled by valves 77 and passed to the next lower sections respectively via lines 78, orifice mixers 79 and lines 80. Raffinate phases from sections 63, 64, and 65 are passed by

action of pumps 81 through lines 82 controlled by valves 83 into the next upper sections respectively by passage through lines 78, orifice mixers 79 and lines 80. Extract phase from section 64 is removed therefrom by pump 85 through line 86, controlled by valve 87. Line 86 connects with line 22 and the mixture is passed into section 65 of extractor 60. Raffinate phase from section 62 is removed therefrom by action of pump 90 through line 91 controlled by valve 92. Line 91 connects with solvent admission pipe 71 and the mixture travels through orifice mixer 73 and line 74 into section 61 of extractor 60.

Final raffinate is removed from extractor 60 via line 94 controlled by valve 95. Intermediate extract phase from extractor 60 passes by action of pump 100 through line 101 controlled by valve 102. The intermediate extract phase may then pass through line 103 and valve 104 into cooler 105 and through line 106 into separator 107 or this equipment may be by-passed by closing valve 104 and opening valve 108. If desired, part of the flow may be through valve 104 and part through valve 108.

When intermediate extract phase passes through valve 104, its temperature is sufficiently reduced by cooler 105 to cause phase separation in separator 107 into an intermediate rejected raffinate and a further extract. When a liquid, normally gaseous solvent is employed, chilling may be accomplished in 105 by vaporization of at least part of the solvent with consequent internal refrigeration. This intermediate rejected raffinate is removed from 107 by pump 110 in line 111 controlled by valve 112. I prefer to return the intermediate raffinate from separator 107 into that zone of extractor 60 wherein the oil being extracted has substantially the same viscosity gravity constant as the rejected raffinate being introduced. The viscosity gravity constant of the intermediate raffinate is usually intermediate that of the final raffinate issuing from extractor 60 via line 94 and that of the oil entering extractor 60 by line 57. Consequently, the intermediate raffinate is preferably introduced into extractor 60 at a point intermediate the introduction of the incoming oil and the removal of the final raffinate. For this purpose line 111 is connected with lines 113, 114, and 115 which are respectively controlled by valves 116, 117, and 118 whereby the intermediate raffinate can be introduced into sections 62, 63 and 64 as desired. Extract phase passes from separator 107 by action of pump 120 through line 121, controlled by valve 122. Line 121 connects with line 101.

Extract phase from separator 107 if valve 104 is open, or extract phase direct from extractor 60 if valve 108 is open, or a mixture of these, passes through line 101 to heater 123 and thence through line 124 into separator 125. Sufficient heat is provided in heater 123 to preferably cause substantially complete vaporization of the solvent from the extract phase. The solvent vapors exit via line 126 controlled by valve 127. Extract freed of solvent is removed by action of pump 130 through line 128 controlled by valve 129 and passes through cooler 131 before introduction into extractor 10 via lines 132 and 38, orifice mixer 39 and line 40. Because this extract phase comprises oil characterized by viscosity gravity constant intermediate that of the raffinate issuing through line 22 and that of the oil entering through line 15, I prefer to introduce the same at an intermediate point in extractor 10, preferably into that zone wherein the oil being ex-

tracted has substantially the same viscosity gravity constant as the extract being introduced.

In the operation of this apparatus, it is desirable in certain instances to maintain sections 26 to 28 of primary extractor 10 at successively decreasing temperatures, but it is also within the purview of my invention to maintain these sections at the same temperature or even at successively increasing temperatures. Similarly, 10 sections 61 to 65 of secondary extractor 60 may also be at successively increasing or decreasing temperatures, or at the same temperature.

The solvent employed for the second extraction may be the same as that used in the primary 15 extraction. In that case, I usually prefer to use higher temperatures in extractor 60 than in the primary extractor 10, although in some instances the same or a lower temperature than that prevailing in the primary extraction may be used 20 in the second extraction.

In order to exemplify the application of my invention to a solvent extraction process involving a pure solvent for the first extraction, followed by a modified solvent for the second extraction, 300 volume percent liquid sulphur dioxide, based upon the amount of oil entering via line 12, is introduced through line 17, orifice mixer 48 and line 49. This selective solvent passes countercurrently in primary extractor 10 with 25 the incoming oil introduced through line 12, orifice mixer 14 and line 15. This oil may be characterized by a viscosity gravity constant of 0.875. The low grade extract containing the major proportion of non-paraffinic fractions and the major 30 proportion of liquid sulphur dioxide is removed from primary extractor 10 through line 19. This low grade extract may be characterized by a viscosity gravity constant of 0.955. The primary raffinate containing a small proportion of liquid 35 sulphur dioxide constitutes the feed for the second extraction and is characterized by a viscosity gravity constant of 0.838. The solvent employed for the second extraction may be modified by one or more of the aforementioned modifying agents; 40 for instance, this solvent may comprise 70% liquid sulphur dioxide, and 30% benzene, and may be used in the proportion of 300 percent of solvent based upon the oil introduced into the system through line 12. It is desirable that the high 45 grade raffinate removed via line 94 will contain substantially all of the paraffinic fractions of low viscosity gravity constant, and it is also desirable that the fractions characterized by low viscosity gravity constant present in the intermediate extract removed from the second extraction 50 via line 101 will be substantially recovered by separation from the extract phase. The final raffinate issuing through line 94 may have a viscosity gravity constant of 0.810 while that of the intermediate extract passing through valve 102 55 may be 0.860.

If desired, valve 104 may be entirely closed, in which event all of the intermediate extract phase passes through line 101 into heater 123 and separator 125, where the solvent is removed. The extract is then cooled in 131 before introduction into primary extractor 10. This introduction is preferably into that zone of 10 where oil of substantially the same viscosity gravity constant is contained. For instance, if the oil passing through line 132 has a viscosity gravity constant of 0.860, I prefer that it be introduced into that portion of extractor 10 wherein the oil being extracted has substantially similar viscosity gravity constant 65 as the extract being introduced in order 70 to

that the equilibrium of the system may be retained.

If the intermediate extract phase from 60 passes through coil 105 and separator 107, the rejected raffinate passing through line 111 may have a viscosity gravity constant of 0.828, for instance. I prefer that this rejected raffinate be returned to that portion of the second extractor 60 wherein the oil being extracted has substantially the same viscosity gravity constant as the rejected 10 raffinate. The extract passing through line 101, heater 123, line 124, separator 125, line 128, cooler 131 and line 132 to the extractor 10 then may have a viscosity gravity constant of 0.863. I prefer to return this extract to a corresponding portion of extractor 10 in the above described manner.

As an example of the temperature conditions which may exist in the above described process, the oil may be introduced into primary extractor 10 via line 12 at 95° F. for countercurrent extraction with liquid sulphur dioxide introduced at 110° F. The primary raffinate thus produced may enter section 65 of column 60 at 80° F. The temperature in 60 may be successively increased until the temperature in section 61 is 120° F. In order to produce adequate phase separation of the intermediate extract phase in separator 107, this mixture may be lowered to 20° F. The intermediate extract phase may be heated to 300° F. in 123 to cause substantially complete removal of sulphur dioxide and benzol in separator 125.

My invention is capable of many modifications. For instance, extractors 10 and 60 may be divided into more or fewer sections. Or, in fact, they may be undivided into sections in which case the oil and solvent can freely flow up and down the columns. My invention may be additionally modified by cooling the extract phase passing through line 19 to reject an intermediate raffinate and by returning this rejected raffinate to that zone in extractor 10 containing oil of substantially the same viscosity gravity constant undissolved in the solvent. Another modification may be to subject 45 the oil flowing through line 132 to extraction with a solvent such as liquid sulphur dioxide in an extractor other than extractor 10.

It is to be understood that the foregoing is merely illustrative of the generic invention, and the examples are not to be taken as limitations thereof, as many modifications of my invention may be made within the scope of the following claims.

I claim:

1. A process for the separation of paraffinic and non-paraffinic fractions from an oil containing the same which comprises countercurrently extracting said oil with a selective solvent, separating a raffinate insoluble in said solvent from the extract phase, separating an intermediate raffinate from said extract phase and introducing said intermediate raffinate into said extraction at that zone wherein oil being extracted has substantially the same viscosity gravity constant as the intermediate raffinate being introduced.

2. A process for the separation of paraffinic and non-paraffinic fractions from an oil containing the same which comprises countercurrently extracting said oil with a selective solvent, separating a raffinate insoluble in said solvent from the extract phase, cooling said extract phase to separate an intermediate raffinate therefrom and introducing said intermediate raffinate into said extraction at a point intermediate the points of 75

introduction of selective solvent and oil entering the system.

3. A process for the separation of paraffinic and non-paraffinic fractions from an oil containing the same which comprises countercurrently extracting said oil with a selective solvent, separating a raffinate insoluble in said solvent from the extract phase, cooling said extract phase to separate an intermediate raffinate therefrom and introducing said intermediate raffinate into said extraction at that zone wherein oil being extracted has substantially the same viscosity gravity constant as said intermediate raffinate being introduced.
4. A process for the separation of paraffinic and non-paraffinic fractions from an oil containing the same which comprises extracting said oil with a selective solvent, separating a raffinate insoluble in said solvent from the extract phase, extracting said raffinate with a selective solvent to produce a final raffinate and an intermediate extract phase, cooling said intermediate extract phase to separate an intermediate raffinate therefrom, removing the intermediate raffinate from the cooled intermediate extract phase, then removing selective solvent from said intermediate extract phase by distillation, cooling the intermediate extract after said distillation and introducing said cooled intermediate extract into said first mentioned extraction at that zone wherein oil being extracted has substantially the same viscosity gravity constant as said intermediate extract being introduced.

5. A method of contact of oil containing paraffinic and non-paraffinic constituents with a selective solvent in which phase separation occurs to produce a raffinate relatively more paraffinic in character and an extract relatively less paraffinic in character than the original oil which method operates in a countercurrent system of contact between the oil and the selective solvent which comprises countercurrently contacting said oil with a selective solvent and thereby forming a raffinate phase and an extract phase, separating said phases, cooling said extract phase and recovering an oil fraction therefrom, said oil fraction having a viscosity gravity constant which is higher than the viscosity gravity constant of oil fractions contained in said raffinate phase and introducing said oil fraction recovered from said extract phase into the extraction system at a point intermediate between the points of introduction in said countercurrent extraction system of the selective solvent and the oil.

6. A method according to claim 5 in which the fraction recovered from the extract phase is introduced into the extraction system at a point in said extraction system wherein the viscosity gravity constant of the oil fractions present at said point is substantially the same as the viscosity gravity constant of said oil fraction recovered from said extract phase.

ULRIC B. BRAY. 30